

July 26, 1960

G. H. JONKER ET AL  
FERROMAGNETIC MATERIAL

2,946,752

Filed Aug. 9, 1956

2 Sheets-Sheet 1



FIG. 1

INVENTORS  
GERARD HEINRICH JONKER  
HENRICUS PETRUS JOHANNES WIJN  
POUL BERNARD BRAUN

BY

*Frederick C. Vogel*  
AGENT

July 26, 1960

G. H. JONKER ET AL

2,946,752

FERROMAGNETIC MATERIAL

Filed Aug. 9, 1956

2 Sheets-Sheet 2



FIG. 2

INVENTORS  
GERARD HEINRICH JONKER  
HENRICUS PETRUS JOHANNES WIJN  
POUL BERNARD BRAUN

BY

*Fred L. Vogel*

AGENT

# United States Patent Office

2,946,752

Patented July 26, 1960

1

2,946,752

## FERROMAGNETIC MATERIAL

Gerard Heinrich Jonker, Henricus Petrus Johannes Wijn, and Poul Bernard Braun, all of Eindhoven, Netherlands, assignors, by mesne assignments, to North American Philips Company, Inc., New York, N.Y., a corporation of Delaware

Filed Aug. 9, 1956, Ser. No. 603,135

Claims priority, application Netherlands Aug. 10, 1955

6 Claims. (Cl. 252—62.5)

Our invention relates to oxidic ferromagnetic materials, to methods of preparing these materials and to bodies made from these materials.

Oxidic ferromagnetic materials which exhibit high values of initial permeability are known in the art. All these materials show a decrease of the initial permeability in a certain frequency range the position of which in the frequency scale is related to the low-frequency value of the initial permeability. The initial permeability decreases in a frequency range the position of which in the frequency scale is higher in proportion as the value of the initial permeability at low-frequency is lower. Thus the cores formed from these materials are not too satisfactory for use at high frequencies.

The principal object of our invention, therefore, is to provide a new and novel class of oxidic ferromagnetic materials the initial permeability of which decreases in a much higher positioned frequency range than in the known materials with an equal low-frequency value of the initial permeability.

Another object of our invention is to provide oxidic ferromagnetic materials which have initial permeabilities of more and often materially more than 2 at frequencies of about 50 mc./s. and often considerably higher frequencies and which exhibit low losses.

Still another object of our invention is to provide oxidic ferromagnetic materials which may serve as materials for magnetic bodies e.g. cores at frequencies of about 50 mc./s. and often considerably higher frequencies.

These and other objects of our invention will be apparent as the specification progresses.

According to our invention we have found a new and novel material which is formed essentially of hexagonal crystals containing about 17.6 mol. percent BaO, 11.8 mol. percent CoO and 70.6 mol. percent Fe<sub>2</sub>O<sub>3</sub>. This material may be considered to have a composition corresponding to the formula Ba<sub>2</sub>Co<sub>2</sub>Fe<sub>24</sub>O<sub>41</sub>. From further investigations it appeared that in the aforesaid formula the Ba-ions may be replaced partly by similar ions, for example Sr-, Ca- and Pb-ions or a combination of these ions, i.e. for not more than one third part. The aforesaid formula may thus be restated as follows:



in which M is at least one metal selected from the group consisting of strontium, calcium, and lead, and the subscript *a* has a value less than 1. These materials have initial permeabilities which do not decrease substantially up to very high frequencies. They have initial permeabilities of more and often materially more than 2 at frequencies of about 50 mc./s. and often considerably higher frequencies. Since they are basically oxidic in nature they are characterized by high ohmic resistances, so that eddy current losses are negligibly small. In addition to having greatly improved initial permeabilities at high frequencies, particularly above 50 mc./s., the

2

materials of our invention exhibit relatively low residual loss factors (tan δ) at frequencies above 50 mc./s.

The novel materials of our invention have a crystal structure of which the unit cell in the hexagonal crystal system has a *c*-axis of about 52.3 Å and an *a*-axis of about 5.9 Å.

We prepare the novel materials of our invention by heating at a temperature of more than 1200° C. a finely divided mixture of metallic oxides in a ratio approximately corresponding to that of the metals in the materials of our invention. Alternatively instead of a metallic oxide we may use a material which forms an oxide when heated. As these oxide-forming materials we may use carbonates, oxalates and acetates of the metals. Moreover, instead of metallic oxides we may use one or more preformed reaction products of at least two of the metallic oxides.

Preferably we prepare the novel materials of our invention by heating to a temperature of more than 1200° C. in an atmosphere containing at least as much oxygen as air, a finely divided mixture of metallic oxides and/or oxide-forming materials and/or reaction products of metallic oxides, in a ratio approximately corresponding to that of the metals in the materials of our invention.

As a preformed reaction product of at least two of the metallic oxides we preferably use an iron-containing reaction product, which has been produced at low temperature, preferably below 1100° C., and which has a crystal structure corresponding with that of the mineral magnetoplumbite, for example Ba<sub>x</sub>Sr<sub>(1-x)</sub>Fe<sub>12</sub>O<sub>19</sub>, where in O  $\leq x \leq 1$ .

If necessary the mixture of oxides and/or equivalent materials may be presintered, usually at a relatively low temperature of about 800° to 1100° C., the presintered material being reground and resintered, several more times if desired, before being subjected to the higher temperatures of the process.

In order to facilitate the sintering operation of our process we may include various flux agents, for example silicates such as pentonite or fluorides such as calcium fluoride in an amount of from 0.25% to 5% in the mixture of the oxides.

Bodies of desired shape may be formed by sintering the starting mixtures directly in the desired shape. Alternatively bodies of desired shape may be formed by regrounding the sintered material of our invention, or the presintered material, molding the resultant powder into the desired shape and sintering the molded product if necessary. A binder such as water, a solution of nitrocellulose or a solution of carboxymethylcellulose may be added to the powdered mixtures before molding if necessary.

In a further embodiment of our invention the finely divided material of our invention is molded to form a body of the desired shape by pressing the relative material together with a binding agent which is capable of being hardened (for example a polyester resin or an ethoxylin resin), followed by hardening the molded body.

Our invention will now be described in greater detail with reference to the following examples and drawing in which:

Fig. 1 is a graph showing the relationship between the values of the real portion of initial permeability,  $\mu'$ , and the values of the loss factor tan δ to frequency for one embodiment of our invention and

Fig. 2 is a graph showing the relationship between the values of the real portion of initial permeability,  $\mu'$ , and the values of the loss factor tan δ to frequency for a second embodiment of our invention.

The relationship between the loss factor tan δ and the real portion of initial permeability,  $\mu'$ , will be apparent

from the following explanation which forms no part of our invention and which is not to be used in any way to limit the scope of our invention:

The term  $\mu'$  as used herein may be explained as follows: A sinusoidally alternating magnetic field with small amplitude will produce a similarly varying inductance in a ferromagnetic body but due to ferromagnetic losses there will be a phase difference between the magnetic field and the inductance. Thus the permeability of the ferromagnetic body,  $\mu$ , may be represented by a complex magnitude  $\mu = \mu' - j\mu''$ . The real portion of permeability,  $\mu'$ , is in phase with the field applied while the other lags in phase by 90° with respect to the applied field. The loss factor "tan  $\delta$ " can then be defined as

$$\tan \delta = \frac{\mu''}{\mu'}$$

#### Example I

A mixture of 62.7 gs. of  $\text{BaCO}_3$ , 197.5 gs. of  $\text{Fe}_2\text{O}_3$  and 25.1 gs. of  $\text{CoCO}_3$  was ground for half an hour with ethyl alcohol in a porcelain ball mill. Subsequent to drying the oxide mixture was heated for 15 hours in air at a temperature of about 1000° C. The reaction product was ground again for half an hour. Then rings were molded therefrom at a pressure of 1000 kgs./cm.<sup>2</sup>, these rings having an outer diameter of about 35 mms. and an inner diameter of about 25 mms. and a height of about 4 mms. These rings were sintered for one hour in oxygen at a temperature of 1280° C. The properties of these sintered rings are indicated in the table under No. 1.

#### Example 1

From a mixture of 62.7 gs. of  $\text{BaCO}_3$ , 200 gs. of  $\text{Fe}_2\text{O}_3$  and 21.3 gs. of  $\text{CoCO}_3$  rings were molded at a pressure of 1000 kgs./cm.<sup>2</sup>; these rings were sintered as in the manner described in Example I. The properties of the sintered rings are indicated in the table under No. 2.

#### Example III

A mixture of 23.0 gs. of  $\text{BaCO}_3$ , 72.5 gs. of  $\text{Fe}_2\text{O}_3$  and 7.95 gs. of  $\text{CoCO}_3$  was ground for half an hour with ethyl alcohol in a porcelain ball mill. The dried mixture was heated for 15 hours in air at 1000° C. and then ground again for half an hour. The powder obtained was heated for one hour in oxygen at 1200° C. This reaction product was reground for one hour. From the powder, rings were molded at a pressure of 1000 kgs./cm.<sup>2</sup> after the addition of a small quantity of a solution of nitro-cellulose as an organic binder. These rings were then heated in oxygen at 1275° C. for three hours, cooled to 1200° C., kept at this temperature for one hour and then cooled to room temperature within 4 hours. The properties of these rings are indicated in the table under No. 3.

#### Example IV

A mixture of 98.7 gs. of  $\text{BaCO}_3$ , 326.6 gs. of  $\text{Fe}_2\text{O}_3$  and 43.3 gs. of  $\text{CoCO}_3$  (with 45.4% by weight of Co) was ground for 16 hours with ethyl alcohol in an iron ball mill. The dried mixture was heated for two hours at 1050° C. and the reaction product was ground again for 16 hours. From the dried powder rings were molded

at a pressure of 1000 kgs./cm.<sup>2</sup> having an outer diameter of about 35 mms., an inner diameter of about 25 mms. and a height of about 4 mms. These rings were sintered for two hours at 1260° C. in oxygen. An X-ray examination proved that the reaction product consisted wholly of crystals with the desired structure. The properties are indicated in the table under No. 4.

#### Example V

10 The compound  $\text{BaFe}_{12}\text{O}_{19}$  was previously produced by heating a mixture of  $\text{BaCO}_3$  and  $\text{Fe}_2\text{O}_3$  in the correct ratio at 1000° C. for 15 hours. Together with  $\text{BaCO}_3$  and  $\text{CoCO}_3$  this product was mixed in the ratio of 2 mols  $\text{BaFe}_{12}\text{O}_{19}$ , 1 mol  $\text{BaCO}_3$  and 2 mols  $\text{CoCO}_3$ , which corresponds to the desired formula  $\text{Ba}_3\text{Co}_2\text{Fe}_{24}\text{O}_{41}$ . The mixture was ground with alcohol in a vibration mill for 4 hours. Rings were molded from this product at a pressure of 1000 kgs./cm.<sup>2</sup>; these rings were fired for one hour at 1270° C. in oxygen. X-ray examination proved that the reaction product consisted wholly of crystals with the desired structure. The properties of the rings are indicated in the table under No. 5.

#### Example VI

25 The compound  $\text{Ba}_{0.6}\text{Sr}_{0.4}\text{Fe}_{12}\text{O}_{19}$  was previously produced by heating a mixture of  $\text{BaCO}_3$ ,  $\text{SrCO}_3$  and  $\text{Fe}_2\text{O}_3$  in the correct ratio for 15 hours at 1000° C. Together with  $\text{BaCO}_3$  and  $\text{CoCO}_3$  this product was mixed in a ratio of 2 mols  $\text{Ba}_{0.6}\text{Sr}_{0.4}\text{Fe}_{12}\text{O}_{19}$ , 1 mol  $\text{BaCO}_3$  and 2 mols  $\text{CoCO}_3$ , which corresponds to the desired compound  $\text{Ba}_{2.2}\text{Sr}_{0.8}\text{Co}_2\text{Fe}_{24}\text{O}_{41}$ . The mixture was ground for 4 hours with alcohol in a vibration mill. Rings were molded from this product at a pressure of 1000 kgs./cm.<sup>2</sup>; these rings were fired for one hour at 1260° C. in oxygen. X-ray examination proved that the reaction product consisted of crystals with the desired structure. The properties of the rings are indicated in the table under No. 6.

#### Example VII

40 A mixture of cobalt carbonate, barium carbonate and ferric oxide in a ratio in accordance with the formula  $\text{Ba}_3\text{Co}_2\text{Fe}_{24}\text{O}_{41}$  was ground for 15 hours with ethyl alcohol in an iron ball mill. The dried mixture was sintered for two hours at 1050° C. and the reaction product was ground again for 15 hours. The dried powder was sintered again for two hours at 1200° C. in a stream of oxygen. This sintered material was finely ground with ethyl alcohol in a vibration mill and then dried. From this powder, rings were molded at a pressure of 200 kgs./cm.<sup>2</sup>, after the addition of a small quantity of a solution of "Araldite" in acetone as an ethoxylin resin, which were heated for eight hours at 130° C. These rings had at a frequency of 260 mc./s. a  $\mu'$  of 2.5.

45 In the following table, in column 2, under the heading of "Main Constituent," chemical formulae are indicated, which were derived from the compositions of the starting mixtures and from the X-ray examinations. All measuring results were obtained by carrying out measurements on rings in a demagnetized state at room temperature by the method described by C. M. van der Burgt, M. Gevers and H. P. J. Wijn in "Philips Technical Review," 14, 245 (1952-1953).

TABLE

| No.    | Main Constituent                                                       | $d$<br>g./cm. <sup>3</sup> | $\rho$<br>$\Omega$ cm. | $\mu'$ low<br>frequency | $\mu'$<br>50 mc./s. | $\mu'$<br>500 mc./s. | Fig. |
|--------|------------------------------------------------------------------------|----------------------------|------------------------|-------------------------|---------------------|----------------------|------|
| 1----- | $\text{Ba}_3\text{Co}_2\text{Fe}_{24}\text{O}_{41}$                    | 4.5                        | 10 <sup>6</sup>        | 12                      | 10                  | 11                   | 1    |
| 2----- | $\text{Ba}_3\text{Co}_2\text{Fe}_{24}\text{O}_{41}$                    | 4.1                        | 10 <sup>6</sup>        | 10                      | 9                   | 11                   | 2    |
| 3----- | $\text{Ba}_3\text{Co}_2\text{Fe}_{24}\text{O}_{41}$                    | 4.1                        | 10 <sup>7</sup>        | 7                       | 7                   | 7                    | 2    |
| 4----- | $\text{Ba}_3\text{Co}_2\text{Fe}_{24}\text{O}_{41}$                    |                            |                        | 21                      | 19                  | 15                   | 2    |
| 5----- | $\text{Ba}_3\text{Co}_2\text{Fe}_{24}\text{O}_{41}$                    |                            |                        | 9.5                     | 9.5                 | 9.6                  | 2    |
| 6----- | $\text{Ba}_{2.2}\text{Sr}_{0.8}\text{Co}_2\text{Fe}_{24}\text{O}_{41}$ |                            |                        | 8.9                     | 8.2                 | 8.9                  | 2    |

The graph of Fig. 1 shows the relationship between the real portion of the initial permeability,  $\mu'$ , and  $\tan \delta$  to frequency for the product of Example II. In this graph the values of  $\mu'$  and  $\tan \delta$  are plotted along the ordinates and the values of the frequencies are plotted along the abscissa.

The graph of Fig. 2 in the same manner shows the relationship between the real portion of the initial permeability,  $\mu'$ , and  $\tan \delta$  to frequency for the product of Example IV.

While we have described our invention in connection with specific embodiments and applications, other modifications thereof will be readily apparent to those skilled in this art without departing from the spirit and scope of the invention as defined in the appended claims.

What is claimed is:

1. A ferromagnetic material consisting essentially of crystals of a composition having the formula



in which M is a metal selected from the group consisting of strontium, calcium, and lead, and  $a$  has a value less than 1, said compound containing as the equivalent a total of 17.6 mol. percent of barium, strontium, calcium and lead oxides, 11.8 mol. percent of CoO and 70.6 mol. percent of  $\text{Fe}_2\text{O}_3$ , said crystals having a structure, the unit cell of which in the hexagonal crystal system has a  $c$ -axis of about 52.3 Å and an  $a$ -axis of about 5.9 Å.

2. A ferromagnetic body having an initial permeability of at least 2 at frequencies of at least 50 mc./sec. consisting essentially of a highly coherent mass of crystals of a composition having the formula:



in which M is a metal selected from the group consisting of strontium, calcium, and lead and  $a$  has a value less than 1, said crystals having a structure, the unit cell of which in the hexagonal system has a  $c$ -axis of 52.3 Å and an  $a$ -axis of about 5.9 Å.

3. A method of producing a ferromagnetic material comprising the steps, forming a finely-divided mixture of oxides in proportions forming upon sintering crystals of a composition having the formula:



in which M is a metal selected from the group consisting of calcium, strontium, and lead and  $a$  has a value less than 1, said crystals having a structure, the unit cell of which in the hexagonal crystal system has a  $c$ -axis of 52.3 Å and an  $a$ -axis of about 5.9 Å; and heating said mixture to a temperature of at least 1200° C. in an atmosphere containing at least as much oxygen as air for a time sufficient to form the crystals.

4. A method of producing a ferromagnetic material comprising the steps, forming a finely-divided mixture of oxides of divalent metals and ferric oxide in proportions forming upon heating crystals having a structure corresponding to the mineral magnetoplumbite; heating said mixture to a temperature below 1100° C. but sufficient to form said crystals; mixing said crystals with oxides forming therewith upon heating crystals of a composition having the formula



in which M is a metal selected from the group consisting of strontium, calcium, and lead, and  $a$  has a value less

than 1, said latter crystals having a structure, the unit cell of which in the hexagonal crystal system has a  $c$ -axis of about 52.3 Å and an  $a$ -axis of about 5.9 Å; heating said latter mixture to a temperature of at least 1200° C. in an atmosphere containing at least as much oxygen as air for a time sufficient to form said latter crystals.

5. A method of producing a ferromagnetic material comprising the steps, forming a finely-divided mixture of oxides in proportions forming upon subsequent heating crystals of a composition having the formula:



in which M is a metal selected from the group consisting of strontium, calcium, and lead, and  $a$  has a value less than 1, said crystals having a structure, the unit cell of which in the hexagonal crystal system has a  $c$ -axis of about 52.3 Å and an  $a$ -axis of about 5.9 Å; heating said mixture to a temperature of about 800° to 1100° C.

20 to substantially react the oxides into forming said composition; finely-dividing said reaction product; and heating said finely-divided reaction product at a temperature of at least about 1200° C. in an atmosphere containing at least as much oxygen as air for a time sufficient to form said crystals.

25 6. A method of making a ferromagnetic body having an initial permeability exceeding at least 2 at a frequency of at least 50 mc./sec. comprising the steps, forming a finely-divided mixture of oxides in proportions forming upon heating crystals of a composition having the formula:  $\text{Ba}_{3-a}\text{M}_a\text{Co}_2\text{Fe}_{24}\text{O}_{41}$ , in which M is a metal selected from the group consisting of strontium, calcium and lead and  $a$  has a value less than 1, said crystals having a structure, the unit cell of which in the hexagonal crystal system has a  $c$ -axis of about 52.3 Å and an  $a$ -axis of about 5.9 Å; compacting said mixture into a body of desired shape and dimensions; and heating said body to a temperature of at least 1200° C. in an atmosphere containing at least as much oxygen as air for a time sufficient to form said crystals.

#### References Cited in the file of this patent

#### UNITED STATES PATENTS

|              |               |                |
|--------------|---------------|----------------|
| 2,659,698    | Berge         | Nov. 17, 1953  |
| 2,723,239    | Harvey        | Nov. 8, 1955   |
| 2,736,708    | Crowley       | Feb. 28, 1956  |
| 2,762,777    | Went          | Sept. 11, 1956 |
| 2,762,778    | Gorter et al. | Sept. 11, 1956 |
| 2,778,803    | Crowley       | Jan. 22, 1957  |
| 50 2,828,264 | Medvedieff    | Mar. 25, 1958  |

#### FOREIGN PATENTS

|            |           |               |
|------------|-----------|---------------|
| 1,100,865  | France    | Apr. 13, 1955 |
| 927,259    | Germany   | May 2, 1955   |
| 55 165,447 | Australia | Oct. 4, 1955  |

#### OTHER REFERENCES

- Erchalk et al.: J. Amer. Chem. Soc., October 1946, pp. 2085-2093.  
 60 Harvey et al.: RCA Review, September 1, 1950, p. 346.  
 "Phillips Technical Review," vol. 13, No. 77, pp. 194-208.  
 "Phillips Technical Review," vol. 18, No. 6, pp. 145-65 154.